



US008455410B2

(12) **United States Patent**  
**Flemming**

(10) **Patent No.:** **US 8,455,410 B2**  
(45) **Date of Patent:** **Jun. 4, 2013**

(54) **LUBRICATING OIL COMPOSITION**

(75) Inventor: **Jonathan P. Flemming**, Oxford (GB)

(73) Assignee: **Infineum International Limited** (GB)

(\*) Notice: Subject to any disclaimer, the term of this patent is extended or adjusted under 35 U.S.C. 154(b) by 9 days.

(21) Appl. No.: **13/290,224**

(22) Filed: **Nov. 7, 2011**

(65) **Prior Publication Data**

US 2012/0111299 A1 May 10, 2012

(30) **Foreign Application Priority Data**

Nov. 8, 2010 (EP) ..... 10190384

(51) **Int. Cl.**  
**C10M 133/16** (2006.01)

(52) **U.S. Cl.**  
USPC ..... **508/287**

(58) **Field of Classification Search**  
USPC ..... 508/287  
See application file for complete search history.

(56) **References Cited**

**U.S. PATENT DOCUMENTS**

7,807,611 B2 10/2010 Kocsis et al.

**OTHER PUBLICATIONS**

R.N. Warrener et al., Evidence for an Olefinic Intermediate in the Configurational Inversion Accompanying . . . , Tetrahedron Letters, vol. 35, No. 15, pp. 2389-239, XP002617351.

*Primary Examiner* — Taiwo Oladapo

(57) **ABSTRACT**

A crankcase lubricating oil composition for an internal combustion engine comprising (A) an oil of lubricating viscosity in a major amount; and, (B) as an additive component in a minor amount one or more, oil-soluble imides derived from a hydrogenated Diels-Alder adduct of a maleic anhydride and a furan, where the imide group has the formula >NR, where R is an aliphatic hydrocarbyl group having 4 to 8 carbon atoms.

**16 Claims, No Drawings**

**1**  
**LUBRICATING OIL COMPOSITION**

RELATED APPLICATION

This application claims priority from European Patent Application No. 10190384.7, filed Nov. 8, 2010, which is incorporated by reference in its entirety.

FIELD OF THE INVENTION

The present invention relates to automotive lubricating oil compositions, more especially to automotive lubricating oil compositions for use in piston engines, especially gasoline (spark-ignited) and diesel (compression-ignited), crankcase lubrication, such compositions being referred to as crankcase lubricants. In particular, although not exclusively, the present invention relates to use of additives with antiwear properties in automotive lubricating oil compositions.

BACKGROUND OF THE INVENTION

A crankcase lubricant is an oil used for general lubrication in an internal combustion engine where an oil sump is situated generally below the crankshaft of the engine and to which circulated oil returns. It is well known to include additives in crankcase lubricants for several purposes.

Phosphorus in the form of dihydrocarbyl dithiophosphate metal salts has been used for many years to provide lubricating oil compositions for internal combustion engines with antiwear properties. The metal may be zinc, an alkali or alkaline earth metal, or aluminium, lead, tin, molybdenum, manganese, nickel or copper. Of these, zinc salts of dihydrocarbyl dithiophosphate (ZDDPs) are most commonly used. However, anticipation of stricter controls on the amount of phosphorus in finished crankcase lubricants has led to the need to provide phosphorus free additives to, at least partially, replace ZDDP in such lubricants.

US 2006/0183647 ('647), now U.S. Pat. No. 7,807,611 B2, addresses this need and describes tartaric compounds in low phosphorus lubricants to provide wear reduction and other properties. The tartaric compounds described include condensation products of a tartaric acid and an amine, specifically described compounds including tartrimides. '647 states that the amines may have the formula  $RR^1NH$  wherein R and  $R^1$  each independently represent H, a hydrocarbon-based radical of 1-150 or 8-30 or 1-30 or 8-150 carbon atoms. '647 specifically describes oleyl tartramide and tridecylpropoxyamine tartramide. Thus, '647 exemplifies the presence of relatively long chain groups on the N imide atom. The molecular weight of the imides is thereby enhanced; this means that more weight of additive is required to provide a defined number of moles of the imide.

SUMMARY OF THE INVENTION

The present invention meets the above problem by providing a phosphorus-free additive in the form of an imide having a short chain hydrocarbyl group, where the imide is derived from a Diels-Alder adduct. The imides of the invention are found to have anti-wear activity comparable to that of the additives described in '647, and at a lower treat rate.

The invention may also be regarded as providing an alternative to the additives described in '647.

In accordance with a first aspect, the present invention provides a crankcase lubricating oil composition for an internal combustion engine comprising, or made by admixing:

(A) an oil of lubricating viscosity in a major amount; and

**2**

(B) as an additive component in a minor amount, one or more oil-soluble imides derived from a hydrogenated Diels-Alder adduct of a maleic anhydride and a furan, where the imide group has the formula  $>NR$ , where R is an aliphatic hydrocarbyl group having 4 to 8, such as 4 to 6, carbon atoms.

According to a second aspect, the present invention provides a method of improving the antiwear properties of a lubricating oil composition which comprises incorporating 10 into the composition in a minor amount one or more additives (B) as defined in the first aspect of the invention.

According to a third aspect, the present invention provides a method of lubricating surfaces of the combustion chamber of an internal combustion chamber during its operation comprising:

(i) providing, in a minor amount, one or more additives (B) as defined in the first aspect of the invention in a major amount of an oil of lubricating viscosity to make a lubricating oil composition, to improve the antiwear properties of the composition;

(ii) providing the lubricating oil composition in the combustion chamber;

(iii) providing a hydrocarbon fuel in the combustion chamber; and

(iv) combusting the fuel in the combustion chamber.

In this specification, the following words and expressions, if and when used, have the meanings ascribed below:

“active ingredients” or “(a.i.)” refers to additive material that is not diluent or solvent;

“comprising” or any cognate word specifies the presence of stated features, steps, or integers or components, but does not preclude the presence or addition of one or more other features, steps, integers, components or groups thereof. The expressions “consists of” or “consists essentially of” or cognates may be embraced within “comprises” or cognates, wherein “consists essentially of” permits inclusion of substances not materially affecting the characteristics of the composition to which it applies;

“hydrocarbyl” means a chemical group of a compound that contains only hydrogen and carbon atoms and that is bonded to the remainder of the compound directly via a carbon atom.

“oil-soluble” or “oil-dispersible”, or cognate terms, used herein do not necessarily indicate that the compounds or additives are soluble, dissolvable, miscible, or are capable of being suspended in the oil in all proportions. These do mean, however, that they are, for example, soluble or stably dispersible in oil to an extent sufficient to exert their intended effect in the environment in which the oil is employed. Moreover, the additional incorporation of other additives may also permit incorporation of higher levels of a particular additive, if desired;

“major amount” means in excess of 50 mass % of a composition;

“minor amount” means less than 50 mass % of a composition;

“TBN” means total base number as measured by ASTM D2896;

“phosphorus content” is measured by ASTM D5185;

“sulfur content” is measured by ASTM D2622; and

“sulfated ash content” is measured by ASTM D874.

Also, it will be understood that various components used, essential as well as optimal and customary, may react under conditions of formulation, storage or use and that the invention also provides the product obtainable or obtained as a result of any such reaction.

Further, it is understood that any upper and lower quantity, range and ratio limits set forth herein may be independently combined.

#### DETAILED DESCRIPTION OF THE INVENTION

The features of the invention relating, where appropriate, to each and all aspects of the invention, will now be described in more detail as follows:

##### Oil of Lubricating Viscosity (A)

The oil of lubricating viscosity (sometimes referred to as "base stock" or "base oil") is the primary liquid constituent of a lubricant, into which additives and possibly other oils are blended, for example to produce a final lubricant (or lubricant composition).

A base oil is useful for making concentrates as well as for making lubricating oil compositions therefrom, and may be selected from natural (vegetable, animal or mineral) and synthetic lubricating oils and mixtures thereof. It may range in viscosity from light distillate mineral oils to heavy lubricating oils such as gas engine oil, mineral lubricating oil, motor vehicle oil and heavy duty diesel oil. Generally the viscosity of the oil ranges from 2 to 30, especially 5 to 20,  $\text{mm}^2\text{s}^{-1}$  at 100° C.

Natural oils include animal and vegetable oils (e.g. castor and lard oil), liquid petroleum oils and hydrorefined, solvent-treated mineral lubricating oils of the paraffinic, naphthenic and mixed paraffinic-naphthenic types. Oils of lubricating viscosity derived from coal or shale are also useful base oils.

Synthetic lubricating oils include hydrocarbon oils such as polymerized and interpolymerized olefins (e.g. polybutylenes, polypropylenes, propylene-isobutylene copolymers, chlorinated polybutylenes, poly(1-hexenes), poly(1-octenes), poly(1-decenes)); alkylbenzenes (e.g. dodecylbenzenes, tetradecylbenzenes, dinonylbenzenes, di(2-ethylhexyl)benzenes); polyphenols (e.g. biphenyls, terphenyls, alkylated polyphenols); and alkylated diphenyl ethers and alkylated diphenyl sulfides and the derivatives, analogues and homologues thereof.

Another suitable class of synthetic lubricating oils comprises the esters of dicarboxylic acids (e.g. phthalic acid, succinic acid, alkyl succinic acids and alkenyl succinic acids, maleic acid, azelaic acid, suberic acid, sebastic acid, fumaric acid, adipic acid, linoleic acid dimer, malonic acid, alkylmalonic acids, alkenyl malonic acids) with a variety of alcohols (e.g. butyl alcohol, hexyl alcohol, dodecyl alcohol, 2-ethylhexyl alcohol, ethylene glycol, diethylene glycol monoether, propylene glycol). Specific examples of these esters include dibutyl adipate, di(2-ethylhexyl)sebacate, di-n-hexyl fumarate, dioctyl sebacate, diisooctyl azelate, diisodecyl azelate, dioctyl phthalate, didecyl phthalate, dieicosyl sebacate, the 2-ethylhexyl diester of linoleic acid dimer, and the complex ester formed by reacting one mole of sebacic acid with two moles of tetraethylene glycol and two moles of 2-ethylhexanoic acid.

Esters useful as synthetic oils also include those made from C<sub>5</sub> to C<sub>12</sub> monocarboxylic acids and polyols, and polyol ethers such as neopentyl glycol, trimethylolpropane, pentaerythritol, dipentaerythritol and tripentaerythritol.

Unrefined, refined and re-refined oils can be used in the compositions of the present invention. Unrefined oils are those obtained directly from a natural or synthetic source without further purification treatment. For example, a shale oil obtained directly from retorting operations, a petroleum oil obtained directly from distillation or ester oil obtained directly from an esterification process and used without further treatment would be unrefined oil. Refined oils are similar

to the unrefined oils except they have been further treated in one or more purification steps to improve one or more properties. Many such purification techniques, such as distillation, solvent extraction, acid or base extraction, filtration and percolation are known to those skilled in the art. Re-refined oils are obtained by processes similar to those used to obtain refined oils applied to refined oils which have been already used in service. Such re-refined oils are also known as reclaimed or reprocessed oils and often are additionally processed by techniques for approval of spent additive and oil breakdown products.

Other examples of base oil are gas-to-liquid ("GTL") base oils, i.e. the base oil may be an oil derived from Fischer-Tropsch synthesised hydrocarbons made from synthesis gas containing H<sub>2</sub> and CO using a Fischer-Tropsch catalyst. These hydrocarbons typically require further processing in order to be useful as a base oil.

For example, they may, by methods known in the art, be hydroisomerized; hydrocracked and hydroisomerized; dewaxed; or hydroisomerized and dewaxed.

Base oil may be categorised in Groups I to V according to the API EOLCS 1509 definition.

When the oil of lubricating viscosity is used to make a concentrate, it is present in a concentrate-forming amount (e.g., from 30 to 70, such as 40 to 60, mass %) to give a concentrate containing for example 1 to 90, such as 10 to 80, preferably 20 to 80, more preferably 20 to 70, mass % active ingredient of an additive or additives, being component (B) above, optionally with one or more co-additives. The oil of lubricating viscosity used in a concentrate is a suitable oleaginous, typically hydrocarbon, carrier fluid, e.g. mineral lubricating oil, or other suitable solvent. Oils of lubricating viscosity such as described herein, as well as aliphatic, naphthenic, and aromatic hydrocarbons, are examples of suitable carrier fluids for concentrates. Concentrates constitute a convenient means of handling additives before their use, as well as facilitating solution or dispersion of additives in lubricating oil compositions. When preparing a lubricating oil composition that contains more than one type of additive (sometimes referred to as "additive components"), each additive may be incorporated separately, each in the form of a concentrate. In many instances, however, it is convenient to provide a so-called additive "package" (also referred to as an "adpack") comprising one or more co-additives, such as described hereinafter, in a single concentrate.

The lubricating oil composition of the invention may be provided, if necessary, with one or more co-additives, such as described hereinafter. This preparation may be accomplished by adding the additive directly to the oil or by adding it in the form of a concentrate thereof to disperse or dissolve the additive. Additives may be added to the oil by any method known to those skilled in the art, either before, at the same time as, or after addition of other additives.

Preferably, the oil of lubricating viscosity is present in an amount of greater than 55 mass %, more preferably greater than 60 mass %, even more preferably greater than 65 mass %, based on the total mass of the lubricating oil composition. Preferably, the oil of lubricating viscosity is present in an amount of less than 98 mass %, more preferably less than 95 mass %, even more preferably less than 90 mass %, based on the total mass of the lubricating oil composition.

The terms "oil-soluble" or "oil-dispersible", or cognate terms, used herein do not necessarily indicate that the compounds or additives are soluble, dissolvable, miscible, or are capable of being suspended in the oil in all proportions. These do mean, however, that they are, for example, soluble or stably dispersible in oil to an extent sufficient to exert their

intended effect in the environment in which the oil is employed. Moreover, the additional incorporation of other additives may also permit incorporation of higher levels of a particular additive, if desired.

The lubricating oil compositions of the invention may be used to lubricate mechanical engine components, particularly in internal combustion engines, e.g. spark-ignited or compression-ignited two- or four-stroke reciprocating engines, by adding the composition thereto. Preferably, they are crank-case lubricants, amongst which may be mentioned heavy duty diesel (HDD) engine lubricants.

The lubricating oil compositions of the invention comprise defined components that may or may not remain the same chemically before and after mixing with an oleaginous carrier. This invention encompasses compositions which comprise the defined components before mixing, or after mixing, or both before and after mixing.

When concentrates are used to make the lubricating oil compositions, they may for example be diluted with 3 to 100, e.g. 5 to 40, parts by mass of oil of lubricating viscosity per part by mass of the concentrate.

The lubricating oil composition of the present invention may contain levels of phosphorus, that are not greater than 1600, preferably not greater than 1200, more preferably not greater than 800, such as not greater than 500, for example, in the range of 200 to 800, or 200 to 500, ppm by mass of phosphorus, expressed as atoms of phosphorus, based on the total mass of the composition. Some of the above may be referred to as low phosphorus oils. In some cases, substantially no phosphorus is present. Preferably, the lubricating oil composition contains not greater than 1000, such as not greater than 800, ppm by mass of phosphorus, expressed as phosphorus atoms.

Typically, the lubricating oil composition may contain low levels of sulfur. Preferably, the lubricating oil composition contains up to 0.4, more preferably up to 0.3, most preferably up to 0.2, mass % sulfur, expressed as atoms of sulfur, based on the total mass of the composition.

Typically, the lubricating oil composition may contain low levels of sulfated ash. Preferably, the lubricating oil composition contains up to 1.0, preferably up to 0.8, mass % sulfated ash, based on the total mass of the composition.

Suitably, the lubricating oil composition may have a total base number (TBN) of between 4 to 15, preferably 5 to 11.

#### Additive Component (B)

(B) may be made by a three-stage process: firstly, a Diels-Alder adduct of a furan and a maleic anhydride is made; secondly, the adduct is catalytically hydrogenated; and finally the product is reacted with a primary amine to convert the anhydride moiety to an imide moiety. The examples of this specification contain an illustrative reaction scheme.

The group R on the imide moiety is, as stated, an aliphatic hydrocarbyl group having 4 to 8 carbon atoms. Preferably R is a straight chain or branched alkyl or alkenyl group. Preferably, R has 4 to less than 7, such as 4 to 6, more preferably 4 or 6, most preferably 4, carbon atoms. A noteworthy example of R is n-butyl. Such additives are found to be oil-soluble or oil-dispersible in the practice of the invention.

(B) may also be defined as a product obtainable by the above process.

Suitably, the additive component (B) is present in an amount of 0.1 to 10 mass %, preferably 0.1 to 5 mass %, more preferably 0.1 to 2 mass %, of the lubricating oil composition, based on the total mass of the lubricating oil composition.

#### Co-Additives

Co-additives, with representative effective amounts, that may also be present, different from additive component (B), are listed below. All the values listed are stated as mass percent active ingredient.

| 10                                  | Additive | Mass %<br>(Broad) | Mass %<br>(Preferred) |
|-------------------------------------|----------|-------------------|-----------------------|
| Ashless Dispersant                  | 0.1-20   | 1-8               |                       |
| Metal Detergents                    | 0.1-15   | 0.2-9             |                       |
| Friction modifier                   | 0-5      | 0-1.5             |                       |
| Corrosion Inhibitor                 | 0-5      | 0-1.5             |                       |
| Metal Dihydrocarbyl Dithiophosphate | 0-10     | 0-4               |                       |
| 15 Anti-Oxidants                    | 0-5      | 0.01-3            |                       |
| Pour Point Depressant               | 0.01-5   | 0.01-1.5          |                       |
| Anti-Foaming Agent                  | 0-5      | 0.001-0.15        |                       |
| Supplement Anti-Wear Agents         | 0-5      | 0-2               |                       |
| Viscosity Modifier (1)              | 0-6      | 0.01-4            |                       |
| Mineral or Synthetic Base Oil       | Balance  | Balance           |                       |

(1) Viscosity modifiers are used only in multi-graded oils.

The final lubricating oil composition, typically made by blending the or each additive into the base oil, may contain from 5 to 25, preferably 5 to 18, typically 7 to 15, mass % of the co-additives, the remainder being oil of lubricating viscosity.

The above mentioned co-additives are discussed in further detail as follows; as is known in the art, some additives can provide a multiplicity of effects, for example, a single additive may act as a dispersant and as an oxidation inhibitor.

A dispersant is an additive whose primary function is to hold solid and liquid contaminations in suspension, thereby passivating them and reducing engine deposits at the same time as reducing sludge depositions. For example, a dispersant maintains in suspension oil-insoluble substances that result from oxidation during use of the lubricant, thus preventing sludge flocculation and precipitation or deposition on metal parts of the engine.

40 Dispersants are usually "ashless", as mentioned above, being non-metallic organic materials that form substantially no ash on combustion, in contrast to metal-containing, and hence ash-forming materials. They comprise a long hydrocarbon chain with a polar head, the polarity being derived from inclusion of e.g. an O, P, or N atom. The hydrocarbon is an oleophilic group that confers oil-solubility, having, for example 40 to 500 carbon atoms. Thus, ashless dispersants may comprise an oil-soluble polymeric backbone.

45 A preferred class of olefin polymers is constituted by polybutenes, specifically polyisobutenes (PIB) or poly-n-butenes, such as may be prepared by polymerization of a C<sub>4</sub> refinery stream.

50 Dispersants include, for example, derivatives of long chain hydrocarbon-substituted carboxylic acids, examples being derivatives of high molecular weight hydrocarbyl-substituted succinic acid. A noteworthy group of dispersants is constituted by hydrocarbon-substituted succinimides, made, for example, by reacting the above acids (or derivatives) with a nitrogen-containing compound, advantageously a polyalkylene polyamine, such as a polyethylene polyamine. Particularly preferred are the reaction products of polyalkylene polyamines with alkenyl succinic anhydrides, such as described in U.S. Pat. Nos. 3,202,678; 3,154,560; 3,172,892; 3,024,195; 3,024,237, 3,219,666; and 3,216,936, that may be post-treated to improve their properties, such as borated (as described in U.S. Pat. Nos. 3,087,936 and 3,254,025) fluorinated and oxylated.

For example, boration may be accomplished by treating an acyl nitrogen-containing dispersant with a boron compound selected from boron oxide, boron halides, boron acids and esters of boron acids.

A detergent is an additive that reduces formation of piston deposits, for example high-temperature varnish and lacquer deposits, in engines; it normally has acid-neutralising properties and is capable of keeping finely divided solids in suspension. Most detergents are based on metal "soaps", that is metal salts of acidic organic compounds.

Detergents generally comprise a polar head with a long hydrophobic tail, the polar head comprising a metal salt of an acidic organic compound. The salts may contain a substantially stoichiometric amount of the metal when they are usually described as normal or neutral salts and would typically have a total base number or TBN (as may be measured by ASTM D2896) of from 0 to 80. Large amounts of a metal base can be included by reaction of an excess of a metal compound, such as an oxide or hydroxide, with an acidic gas such as carbon dioxide. The resulting overbased detergent comprises neutralised detergent as an outer layer of a metal base (e.g. carbonate) micelle. Such overbased detergents may have a TBN of 150 or greater, and typically of from 250 to 500 or more.

Detergents that may be used include oil-soluble neutral and overbased sulfonates, phenates, sulfurized phenates, thiophosphonates, salicylates, and naphthenates and other oil-soluble carboxylates of a metal, particularly the alkali or alkaline earth metals, e.g. sodium, potassium, lithium, calcium and magnesium. The most commonly-used metals are calcium and magnesium, which may both be present in detergents used in a lubricant, and mixtures of calcium and/or magnesium with sodium. Detergents may be used in various combinations, for example with salicylate detergents or without salicylate detergents.

Friction modifiers include glyceryl monoesters of higher fatty acids, for example, glyceryl mono-oleate; esters of long chain polycarboxylic acids with diols, for example, the butane diol ester of a dimerized unsaturated fatty acid; oxazoline compounds; and alkoxylated alkyl-substituted monoamines, diamines and alkyl ether amines, for example, ethoxylated tallow amine and ethoxylated tallow ether amine.

Other known friction modifiers comprise oil-soluble organo-molybdenum compounds. Such organo-molybdenum friction modifiers also provide antioxidant and antiwear credits to a lubricating oil composition. Suitable oil-soluble organo-molybdenum compounds have a molybdenum-sulfur core. As examples there may be mentioned dithiocarbamates, dithiophosphates, dithiophosphinates, xanthates, thioxanthates, sulfides, and mixtures thereof. Particularly preferred are molybdenum dithiocarbamates, dialkyl dithiophosphates, alkyl xanthates and alkylthioxanthates. The molybdenum compound is dinuclear or trinuclear.

One class of preferred organo-molybdenum compounds useful in all aspects of the present invention is tri-nuclear molybdenum compounds of the formula  $Mo_3S_kL_nQ_z$  and mixtures thereof wherein L are independently selected ligands having organo groups with a sufficient number of carbon atoms to render the compounds soluble or dispersible in the oil, n is from 1 to 4, k varies from 4 through to 7, Q is selected from the group of neutral electron donating compounds such as water, amines, alcohols, phosphines, and ethers, and z ranges from 0 to 5 and includes non-stoichiometric values. At least 21 total carbon atoms should be present among all the ligands' organo groups, such as at least 25, at least 30, or at least 35 carbon atoms.

The molybdenum compounds may be present in a lubricating oil composition at a concentration in the range 0.1 to 2 mass %, or providing at least 10 such as 50 to 2,000 ppm by mass of molybdenum atoms.

Preferably, the molybdenum from the molybdenum compound is present in an amount of from 10 to 1500, such as 20 to 1000, more preferably 30 to 750, ppm based on the total weight of the lubricating oil composition. For some applications, the molybdenum is present in an amount of greater than 10 500 ppm.

Anti-oxidants are sometimes referred to as oxidation inhibitors; they increase the resistance of the composition to oxidation and may work by combining with and modifying peroxides to render them harmless, by decomposing peroxides, or by rendering an oxidation catalyst inert. Oxidative deterioration can be evidenced by sludge in the lubricant, varnish-like deposits on the metal surfaces, and by viscosity growth.

They may be classified as radical scavengers (e.g. sterically 20 hindered phenols, secondary aromatic amines, and organo-copper salts); hydroperoxide decomposers (e.g., organosulfur and organophosphorus additives); and multifunctionals (e.g. zinc dihydrocarbyl dithiophosphates, which may also 25 function as anti-wear additives, and organo-molybdenum compounds, which may also function as friction modifiers and anti-wear additives).

Examples of suitable antioxidants are selected from copper-containing antioxidants, sulfur-containing antioxidants, aromatic amine-containing antioxidants, hindered phenolic 30 antioxidants, dithiophosphates derivatives, metal thiocarbamates, and molybdenum-containing compounds.

Dihydrocarbyl dithiophosphate metals salts are frequently used as antiwear and antioxidant agents. The metal may be an alkali or alkaline earth metal, or aluminium, lead, tin, zinc 35 molybdenum, manganese, nickel or copper. Zinc salts are most commonly used in lubricating oil such as in amounts of 0.1 to 10, preferably 0.2 to 2, mass %, based upon the total mass of the lubricating oil compositions. They may be prepared in accordance with known techniques by first forming a dihydrocarbyl dithiophosphoric acid (DDPA), usually by 40 reaction of one or more alcohols or a phenol with  $P_2S_5$ , and then neutralising the formed DDPA with a zinc compound. For example, a dithiophosphoric acid may be made by reaction with mixtures of primary and secondary alcohols. Alternatively, multiple dithiophosphoric acids can be prepared 45 where the hydrocarbyl groups on one acid are entirely secondary in character and the hydrocarbyl groups on the other acids are entirely primary in character. To make the zinc salt, any basic or neutral zinc compound could be used but the oxides, hydroxides and carbonates are most generally employed. Commercial additives frequently contain an excess of zinc due to use of an excess of the basic zinc compound in the neutralisation reaction.

Such metal salts may suitably be employed in combination 50 with additive component(s) (B), for example where (B) contains 100 mole % of alcohol(s) ROH and constitutes at least 50 mole % of the total ZDDP content, of whatever type, in the lubricating oil composition.

Anti-wear agents reduce friction and excessive wear and 55 are usually based on compounds containing sulfur or phosphorous or both, for example that are capable of depositing polysulfide films on the surfaces involved. Noteworthy are the dihydrocarbyl dithiophosphates, such as the zinc dialkyl dithiophosphates (ZDDP's) discussed herein.

Examples of ashless anti-wear agents include 1,2,3-triazoles, benzotriazoles, thiadiazoles, sulfurised fatty acid esters, and dithiocarbamate derivatives.

Rust and corrosion inhibitors serve to protect surfaces against rust and/or corrosion. As rust inhibitors there may be mentioned non-ionic polyoxyalkylene polyols and esters thereof, polyoxyalkylene phenols, and anionic alkyl sulfonic acids.

Pour point depressants, otherwise known as lube oil flow improvers, lower the minimum temperature at which the oil will flow or can be poured. Such additives are well known. Typical of these additive are C<sub>8</sub> to C<sub>18</sub> dialkyl fumarate/vinyl acetate copolymers and polyalkylmethacrylates.

Additives of the polysiloxane type, for example silicone oil or polydimethyl siloxane, can provide foam control.

A small amount of a demulsifying component may be used. A preferred demulsifying component is described in EP-A-330,522. It is obtained by reacting an alkylene oxide with an adduct obtained by reaction of a bis-epoxide with a polyhydric alcohol. The demulsifier should be used at a level not exceeding 0.1 mass % active ingredient. A treat rate of 0.001 to 0.05 mass % active ingredient is convenient.

Viscosity modifiers (or viscosity index improvers) impart high and low temperature operability to a lubricating oil. Viscosity modifiers that also function as dispersants are also known and may be prepared as described above for ashless dispersants. In general, these dispersant viscosity modifiers are functionalised polymers (e.g. interpolymers of ethylene-propylene post grafted with an active monomer such as maleic anhydride) which are then derivatised with, for example, an alcohol or amine.

The lubricant may be formulated with or without a conventional viscosity modifier and with or without a dispersant viscosity modifier. Suitable compounds for use as viscosity modifiers are generally high molecular weight hydrocarbon polymers, including polyesters. Oil-soluble viscosity modifying polymers generally have weight average molecular weights of from 10,000 to 1,000,000, preferably 20,000 to 500,000, which may be determined by gel permeation chromatography or by light scattering.

## EXAMPLES

The invention will now be particularly described in the following examples which are not intended to limit the scope of the claims hereof.

### Synthesis of Diels-Alder Derivatives

#### (i) Reaction of Furan and Maleic Anhydride

Maleic anhydride (1 eq., 1 wt) was added to a solution of furan (5.4 eq., 3.7 wt) in diethyl ether (2 vols). The reaction mixture was stirred at ambient temperature for six hours when a white solid had crystallised. The solid was filtered and washed with diethyl ether (3×2 vols) and then dried under vacuum. The reaction that occurred is represented as:



#### (ii) Hydrogenation

10% palladium on carbon (1 mole %, 0.064 wt) was added to a solution of the solid 1 of step (i) (1 eq., 1 wt) in acetone (10 vols). The reaction mixture was stirred at ambient temperature under a 4 bar hydrogen atmosphere. After one hour,

the resulting mixture was filtered through celite and the solvent removed under pressure to yield the product as:



#### (iii) Synthesis of Imide

n-Butylamine (1 eq., 0.59 vols) was added to a solution of the product 2 of step (ii) (1 eq., 1 wt) and triethylamine (3.6 e.g., 3.0 vols) in toluene (15 vols). The reaction mixture was heated to reflux and the water produced collected in a Dean and Stark trap. When water production ceased, the mixture was cooled to ambient temperature and the solvent removed under reduced pressure yielding an imide—Example 1—(4-n-butyl-10-oxa-4-azatricyclo[5.2.1.0<sup>2,6</sup>]decane-3,5-dione) as depicted below 3:



For convenience, the product will be referred to by the shorthand name of n-butyliimide.

### Lubricating Oil Compositions

Two sets of oil compositions were prepared.

A first set comprised heavy duty diesel Oil X including respectively n-butyliimide (0.5 or 1 mass %); or, as a comparison, tridecylpropoxyamine tartrimide (1 mass %); or ZDDP (0.75 mass %, 600 ppm by mass P).

Oil X contained additive base stock, detergents, dispersants, antioxidant, polyisobutene, antifoam, base stock, and viscosity modifier.

A second set comprised Oils Y, Y<sup>I</sup> and Y<sup>II</sup> having the mass % formulations:

| Oil             | Base Stock | Additive Base Stock | Detergent | n-Butyliimide |
|-----------------|------------|---------------------|-----------|---------------|
| Y               | 80         | 20                  | —         | —             |
| Y <sup>I</sup>  | 80         | 15.4                | 4.60      | —             |
| Y <sup>II</sup> | 80         | 14.4                | 4.60      | 1             |

### Testing and Results

A high frequency reciprocating rig (ex PCS Instruments) was used to evaluate the antiwear properties of each of the above oil compositions by measuring the HFRR ball x-axis wear scar in mm. Experimentation was carried out under the following conditions:

60 minutes at 100° C.

20 Hz reciprocation of 1 mm stroke length

800 g load using standard equipment manufacturer supplied steel substrates.

A control was carried out on Oil X without additives.

## 11

Results are set out in the tables below.

TABLE 1

| Oil                                        | Wear Scar (mm) |
|--------------------------------------------|----------------|
| X (control)                                | 0.340          |
| X + n-butylimide (0.5%)                    | 0.275          |
| X + n-butylimide (1.0%)                    | 0.264          |
| X + tridecylpropoxyamine tartramide (1.0%) | 0.2865         |
| X + ZDDP (0.75%)                           | 0.268          |

The results show that the n-butylimide-containing oil was significantly better than the control in antiwear performance and was even better than or comparable with the ZDDP- and with the tridecylpropoxyamine tartramide-containing oils.

TABLE 2

| Oil                                                     | Wear Scar (mm) |
|---------------------------------------------------------|----------------|
| Y (control)                                             | 0.336          |
| Y <sup>I</sup> (control & detergent)                    | 0.349          |
| Y <sup>II</sup> (control & detergent & 1% n-butylimide) | 0.235          |

The results show that the imide has a significant effect as an antiwear additive, and had superior antiwear activity in comparison with the detergent componentry.

The invention claimed is:

1. A crankcase lubricating oil composition for an internal combustion engine comprising, or made by admixing:
  - (A) an oil of lubricating viscosity in a major amount; and
  - (B) as an additive component in a minor amount, one or more oil-soluble imides derived from a hydrogenated Diels-Alder adduct of a maleic anhydride and a furan, where the imide group comprises the group >NR, where R is an aliphatic hydrocarbyl group having 4 to 8 carbon atoms.
2. A composition as claimed in claim 1 wherein the hydrocarbyl group is a straight chain or branched alkyl or alkenyl group.
3. A composition as claimed in claim 1 wherein the hydrocarbyl group has 4 to 7 carbon atoms.
4. A composition as claimed in claim 3 wherein the hydrocarbyl group has 4 to 6 carbon atoms.
5. A composition as claimed in claim 2 wherein the hydrocarbyl group has 4 to 7 carbon atoms.
6. A composition as claimed in claim 5 wherein the hydrocarbyl group has 4 to 6 carbon atoms.

7. A composition as claimed in claim 1 wherein the hydrocarbyl group is a butyl group.

8. A composition as claimed in claim 7 wherein the hydrocarbyl group is n-butyl.

9. A composition as claimed in claim 1 wherein the composition has a sulfated ash value of up to 1.0 mass % and a sulfur content of up to 0.4 mass %.

10. A composition as claimed in claim 1 wherein the composition contains other additive components, different from (B), selected from one or more of ashless dispersants, metal detergents, corrosion inhibitors, antioxidants, pour point depressants, antiwear agents, friction modifiers, demulsifiers, antifoam agents and viscosity modifiers.

11. A composition as claimed in claim 1 having not greater than 1600 ppm by mass of phosphorus, expressed as phosphorus atoms.

12. A composition as claimed in claim 11 having not greater than 1200 ppm by mass of phosphorus, expressed as phosphorus atoms.

13. A composition as claimed in claim 12 having not greater than 800 ppm by mass of phosphorus, expressed as phosphorus atoms.

14. A composition of claimed in claim 13 having not greater than 500 ppm by mass of phosphorus, expressed as atoms of phosphorus.

15. A method of improving the antiwear properties of a lubricating oil composition which comprises incorporating into the composition in a minor amount one or more one or more oil-soluble imides derived from a hydrogenated Diels-Alder adduct of a maleic anhydride and a furan, where the imide group comprises the group >NR, where R is an aliphatic hydrocarbyl group having 4 to 8 carbon atoms.

16. A method of lubricating surfaces of the combustion chamber of an internal combustion chamber during its operation comprising:

providing, in a minor amount, one or more oil-soluble imides derived from a hydrogenated Diels-Alder adduct of a maleic anhydride and a furan, where the imide group comprises the group >NR, where R is an aliphatic hydrocarbyl group having 4 to 8 carbon atoms, in a major amount of an oil of lubricating viscosity to make a lubricating oil composition;

(ii) providing the lubricating oil composition in the combustion chamber;

(iii) providing a hydrocarbon fuel in the combustion chamber; and

(iv) combusting the fuel in the combustion chamber.

\* \* \* \* \*